

3,210,278

METALLIC HALIDE THIOUREA COMPOUNDS  
 Jack Ryer, East Brunswick, Paul M. Kerschner, Trenton,  
 and Walter C. Bradbury, Newark, N.J., assignors to  
 Cities Service Oil Company, a corporation of Delaware  
 No Drawing. Filed Dec. 26, 1962, Ser. No. 247,363  
 18 Claims. (Cl. 252—46.4)

This application is a continuation-in-part of application Serial No. 502, filed January 5, 1960, now abandoned.

This invention relates to new organo metallic compounds and more particularly to divalent metal halide organo metal complexes of thiourea and to a method for preparing the same.

There has been in recent years a growing interest in the combination of organic radicals and metals to provide new and unique structures having a variety of characteristics and properties which serve a multitude of purposes. New organo-metallic structures have been found particularly useful as catalysts, solvents, chemical intermediates, additives and in many other applications.

The present invention is directed to a new series of compounds of this type; more particularly metallic halide-thiourea complexes having the general structure



wherein X is a halogen selected from the group consisting of chlorine, bromine and iodine, M is a divalent metal selected from the group consisting of zinc, cadmium and manganese, R and R' represent a substituent selected from the group consisting of hydrogen, alkyl having from 3 to 20 carbon atoms, alicyclic having from 6 to 20 carbon atoms, amine substituted acyclic having from 2 to 11 carbon atoms, aralkyl having from 7 to 20 carbon atoms, and aryl, and R'' and R''' represent a substituent selected from the group consisting of alkyl having from 3 to 20 carbon atoms, alicyclic having from 6 to 20 carbon atoms, amine substituted acyclic having from 2 to 11 carbon atoms, aralkyl having from 7 to 20 carbon atoms, and aryl.

The divalent metal halide-thiourea compounds of the present invention are prepared by first synthesizing an intermediate N, N' or N, N, N', N', substituted thiourea which is thereafter reacted with a divalent metal halide to produce a complex having the structure shown in the general formula. Quite unexpectedly these new compounds have been found to be most effective as extreme pressure additives when utilized in small amounts in various lubricating compositions which include synthetic, as well as mineral oil base lubricants.

In preparing lubricant compositions with the extreme pressure agents of the present invention it has been found that an amount of additive of from 0.05% to about 15.0% by weight makes a most satisfactory lubricant composition. Preferably, the agent or extreme pressure additive will be used in an amount of from 0.1 to about 10% by weight of the base lubricant material. In preparing these new lubricant compositions, it has been found that a wide variety of both mineral oil and synthetic base stocks, including mixtures of the same, can be used. Suitable mineral oil base materials include 100 and 200 neutral oils, light and heavy intermediate mineral oils, bright stock and as well as combinations of the foregoing. If a synthetic base material is used diesters, polyesters, silicones, silicates, fluorocarbons, phosphates, polyglycols and polyphenyl ethers and mixtures of the same may be used.

In carrying out the preparation of these extreme pressure compounds according to the method of this invention two mols of an amine are reacted with one mol of carbon disulfide in the presence of a suitable hydrocarbon solvent such as benzene, toluene, xylene, propylbenzene or the like, under reflux conditions determined by the particular solvent utilized. As the reaction between the amine and carbon disulfide progresses hydrogen sulfide is evolved. The reaction is completed when hydrogen sulfide ceases to be evolved. The substituted thiourea product obtained is dissolved in an alcohol solvent such as ethanol, propanol, isopropanol, butanol, isobutanol, or the like, and heated to boiling. To this solution a hot alcohol solution of a selected metal halide is added. A substantially instantaneous reaction occurs producing a divalent metal halide substituted thiourea complex. The latter reaction is carried out in a molar ratio of approximately one mol of substituted thiourea to one-half mol of the metallic halide. If this reaction is not immediate on mixing, a gentle reflux may be applied at a temperature dependent on the solvent utilized. In selecting the latter, it is essential that the solution of the substituted thiourea and the solution of the metallic halide be mutually miscible. If reflux is carried out, either in the initial reaction leading to the preparation of the substituted thiourea or in the reaction of the latter with the metallic halide, periods of up to 12 hours or more may be necessary to bring about a completed reaction.

In preparing the substituted thiourea it has been found that aliphatic amines having from 3 to 20 carbon atoms, either straight chain or branched chain, as well as cyclic, aromatic or substituted aromatic amines, or mixtures thereof may be used. The amine may be a primary or secondary amine and may include unsaturation in a chain or ring structure. Suitable amines for preparing the intermediate substituted thiourea include the following: propylamine, butylamine, pentylamine, hexylamine, cyclohexylamine, heptylamine, octylamine, nonylamine, decylamine, undecylamine, dodecylamine, tridecylamine, tetradecylamine, pentadecylamine, hexadecylamine, benzylamine, heptadecylamine, octadecylamine, nonadecylamine, eicosylamine, diethylamine, N-ethylpropylamine, dipropylamine, N-propylbutylamine, dibutylamine, N-butylpentylamine, dipentylamine, N-pentylhexylamine, dihexylamine, N-hexylheptylamine, diheptylamine, N-heptyloctylamine, dioctylamine, N-octylnonylamine, dinonylamine, N-nonyldecylamine, didecylamine, N-methylpentylamine, N-methylhexylamine, N-ethylpentylamine, N-ethylhexylamine, N-propylpentylamine, N-propylhexylamine, N-butylhexylamine, N-methylheptylamine, N-ethylheptylamine, N-propylheptylamine, N-butylheptylamine, N-methyloctylamine, N-ethyloctylamine, N-propyloctylamine, N-butyloctylamine, N-pentyloctylamine, N-methylnonylamine, N-ethylnonylamine, N-propylnonylamine, N-butylnonylamine, N-pentylnonylamine, N-hexylnonylamine, N-methyldecylamine, N-ethyldecylamine, N-propyldecylamine, N-butyldecylamine, N-pentyldecylamine, N-hexyldecylamine, N-heptyldecylamine, phenylbutylamine, and N-octydecylamine. Lower molecular weight acyclic polyamines such as di-N-butylaminopropylamine, ethylenediamine, diethylenetriamine, triethylenetriamine, and triethylenetetramine may be used.

In the foregoing general formula the amine residues are represented by R, R', R'' and R'''. These substituents may of course be similar or dissimilar depending on the amines selected in preparing the aminothiourea. If two mols of a primary amine are used, R and R' will represent hydrogen with R'' and R''' representing the residues of the amine chain. If secondary amines of a mixture of secondary and primary amines are used, R, R', R'' and R''' will represent the residues of the respective amines used.

The divalent metal halide selected for reaction with the substituted thiourea will be a halide of a metal selected from the group consisting of zinc, cadmium and manganese. It is preferred that the halogen be either chlorine, bromine or iodine. As previously indicated, a hot alcoholic solution of the divalent metal halide is prepared and reacted with an alcoholic solution or equivalent solvent solution of the substituted thiourea. After this reaction has been completed excess solvent is removed from the reaction zone by distillation. Trace residues of unreacted thiourea may be removed from the reaction zone by distillation under vacuum.

The examples which follow will provide a more complete understanding of the new compounds and their manner of preparation, as well as the lubricant compositions in which these compounds are used.

#### EXAMPLE 1

To a one liter flask equipped with a stirrer, reflux condenser and dropping funnel, 398 gms. (2 mols) of Primene 81R (a Rohm & Haas mixed primary amine product) the residue formula of which is



and 100 ml. toluene were added. 76 gms. (1 mol) of carbon disulfide was added dropwise to the flask. The temperature was maintained in the range of from 20 to 30° C. during addition of the carbon disulfide. After the carbon disulfide was added, the mixture was refluxed at a temperature of 100 ± 10° C. and maintained at this temperature for 12 hours. After this time no further evolution of  $\text{H}_2\text{S}$  was noted. The reaction mixture was cooled to room temperature and the toluene solvent removed from the reaction flask by distillation with trace removal of toluene and unreacted amine being accomplished under vacuum. A 99.3% yield of the desired compound  $\text{S}=\text{C}[\text{NHC}(\text{CH}_3)_2(\text{C}_{9-11}\text{H}_{19-23})_2]$  was obtained. One mol of this product (440 gms.) was dissolved in 50 ml. of isopropyl alcohol and heated to boiling. 68 gms. (0.5 mol) of zinc chloride, dissolved in a minimum amount of hot isopropyl alcohol, was slowly added with stirring to the boiling alcoholic disubstituted thiourea solution. The mixture was allowed to cool to room temperature and excess isopropyl alcohol was stripped by distillation from the reaction product complex. An 88% yield of the complex



was obtained. The compound is a liquid, reddish brown in color and has a molecular weight of 1016. An analysis of this compound showed 5.9% by weight of zinc and 5.3% by weight of sulfur. The calculated weight percentage for zinc and sulfur are 6.4% and 6.3% respectively. The effectiveness of this compound as an extreme pressure additive is demonstrated in the table which follows wherein the compound is identified as D.

#### EXAMPLE 2

Following the procedure set forth in Example 1 dichlorobis-N,N'-dicyclohexylthioureazinc was prepared by first reacting 198 gm. (2.0 mol) cyclohexylamine with 76 gm. (1.0 mol) carbon disulfide in the presence of ethanol and a small amount of potassium hydroxide. After evolution of hydrogen sulfide ceased excess ethanol was removed from the reaction zone by distillation. An isopropyl alcohol solution of 68 gms. (0.5 mol) zinc chloride was added to a boiling isopropyl alcohol solution N, N' dicyclohexylthiourea. Excess alcohol was removed from the reaction mixture leaving a light colored liquid product of dichlorobis-N,N'-dicyclohexylthioureazinc ( $\text{Cl}_2\text{Zn}[\text{S}=\text{C}(\text{NHC}_6\text{H}_{11})_2]_2$ ).

#### EXAMPLE 3

Following the procedure set forth in Example 1 dichlorobis-N,N'-di-n-butylthioureazinc was prepared by reacting two mols of n-butylamine with one mol of carbon di-

sulfide to yield an N,N'-di-n-butylthiourea intermediate which was thereafter reacted with one-half mol of an alcoholic solution of zinc chloride to yield dichlorobis-N,N'-n-butylthioureazinc ( $\text{Cl}_2\text{Zn}[\text{S}=\text{C}(\text{NHC}_4\text{H}_9)_2]_2$ ). This compound has a molecular weight of 512 and contained 12.9% zinc. The effectiveness of this compound as an extreme pressure additive is demonstrated in the table which follows, wherein the compound is identified as A.

#### EXAMPLE 4

Two mols of n-hexylamine were reacted according to the method of Example 1 with one mol of carbon disulfide under reflux conditions in the presence of approximately 100 ml. of toluene until the evolution of hydrogen sulfide ceased. The N,N'-di-n-hexylthiourea obtained when reacted with a hot isopropyl alcohol solution of zinc chloride yielded dichlorobis-N,N'-di-n-hexylthioureazinc ( $\text{Cl}_2\text{Zn}[\text{S}=\text{C}(\text{NHC}_6\text{H}_{13})_2]_2$ ) having a molecular weight of 616. This compound analyzed as follows—percent zinc by weight 9.7, percent sulfur by weight 9.2.

#### EXAMPLE 5

Two mols of di-n-butylaminopropylamine



were reacted according to the method of Example 1 with one mol of carbon disulfide under reflux conditions in the presence of toluene until the evolution of hydrogen sulfide ceased. One mol of the N,N'-di(n-butylaminopropyl) thiourea obtained was reacted with a hot isopropyl alcohol solution of one-half mol of zinc chloride to yield dichlorobis-N,N'-di-(di-n-butylaminopropyl) thioureazinc ( $\text{Cl}_2\text{Zn}[\text{S}=\text{C}(\text{NHC}_3\text{H}_9\text{N}(\text{C}_4\text{H}_9)_2)_2]_2$ ). This compound has a molecular weight of 976 and analyzed as follows:

Percent S: Found, 6.3; calculated, 6.6.

#### EXAMPLE 6

Two mols of octadecylamine were reacted according to the method of Example 1 with one mol of carbon disulfide under reflux conditions in the presence of toluene until the evolution of hydrogen sulfide ceased. The N,N'-di-octadecylthiourea obtained when reacted with a hot isopropyl alcohol solution of zinc chloride in the molar ratio of 2:1 yielded dichlorobis-N,N'-di-octadecylthioureazinc ( $\text{Cl}_2\text{Zn}[\text{S}=\text{C}(\text{NHC}_{18}\text{H}_{37})_2]_2$ ) having a molecular weight of 1296 and the following amounts of zinc and sulfur:

Percent Zn: Found, 5.0; calculated, 5.0. Percent S: Found, 5.0; calculated, 5.0.

#### EXAMPLE 7

Two mols of dodecylamine were reacted according to the foregoing examples with one mol of carbon disulfide under reflux conditions in the presence of toluene until the evolution of hydrogen sulfide ceased. The N,N'-di-dodecylthiourea obtained was then reacted with a hot isopropyl alcohol solution of zinc chloride to yield dichlorobis-N,N'-di-dodecylthioureazinc



having a molecular weight of 960, 6.9% by weight of zinc and 6.2% by weight of sulfur. The calculated values for this compound of zinc and sulfur are 6.8 and 6.7 respectively. The compound is identified as B in the table which follows.

#### EXAMPLE 8

Two mols of Armeen-C (a mixed aliphatic amine product of the Armour Co. having the formula



were reacted according to the method of Example 1 with one mol of carbon disulfide under reflux conditions until the evolution of hydrogen sulfide ceased. The mixed dialkyl substituted thiourea obtained was reacted with a hot isopropyl alcohol solution of zinc chloride in a molar

ratio of 2:1 to yield a zinc chloride complex of the mixed dialkyl substituted thiourea.

#### EXAMPLE 9

Two mols of phenylamine were reacted according to the method described in the foregoing examples with one mol of carbon disulfide under reflux conditions in the presence of xylene until no further hydrogen sulfide evolution was noted. After removal of solvent an alcohol solution of N,N'-diphenylthiourea was reacted with one-half mol of zinc chloride to yield dichlorobis-N,N'-diphenylthioureazinc ( $\text{Cl}_2\text{Zn}[\text{S}=\text{C}(\text{NHC}_6\text{H}_5)_2]_2$ ).

#### EXAMPLE 10

Two mols of oleylamine were reacted according to the method of Example 1 with one mol of carbon disulfide under reflux conditions in the presence of toluene until the evolution of hydrogen sulfide was completed. The N,N'-dioleylthiourea obtained was thereafter reacted in the manner previously described with zinc chloride to yield dichlorobis-N,N'-dioleylthioureazinc



This compound is identified as C in the table following.

#### EXAMPLE 11

Two mols of Primene JM-T (a Rohm & Haas mixed amine commercially available product having the following carbon chain structure— $(-\text{C}(\text{CH}_3)_2(\text{C}_{15-19}\text{H}_{31-39})$ ) was reacted according to the method previously described with one mol of carbon disulfide to yield a disubstituted thiourea. This intermediate was then reacted with an alcohol solution of zinc chloride in a molar ratio of 2:1 to yield a dichlorothioureazinc complex identified as compound E in the table.

#### EXAMPLE 12

Two mols of Primene 81R were reacted with one mol of carbon disulfide to yield an intermediate disubstituted thiourea which was thereafter reacted with an alcoholic solution of cadmium chloride in the manner previously described to yield the dichlorocadmium complex of the disubstituted thiourea. The product obtained 4.6% cadmium by weight and 3.8% sulfur.

#### EXAMPLE 13

Two mols of Primene 81R were reacted with one mol of carbon disulfide to yield an N,N' disubstituted thiourea which was thereafter reacted in a molar ratio of 2:1 with manganese chloride according to the method described above to yield the dichloromanganese complex of the disubstituted thiourea. This product is identified as compound F in the table.

#### EXAMPLE 14

To a one liter flask equipped with a stirrer, reflux condenser and dropping funnel, 2 mols of Primene 81R and 100 ml. of toluene are added. One mol of carbon disulfide is added dropwise to the flask. The temperature is maintained within the range of 20 to 30° C. during the addition of the carbon disulfide. After the addition, the mixture is refluxed at a temperature of 100  $\pm 10$ ° C. and maintained at this temperature until reaction mixture is cooled to room temperature and the toluene solvent is removed by distillation in vacuo with trace removal of toluene and unreacted amine. Two mols of this product is reacted with one mol of zinc bromide dissolved in a minimum amount of hot isopropyl alcohol. The mixture is cooled to room temperature and excess alcohol stripped from the reaction product. The dibromozinc complex of the disubstituted thiourea is thereby obtained.

#### EXAMPLE 15

To a one liter flask equipped with a stirrer, reflux condenser and dropping funnel, 186 gms. (2 mols) of

aniline and 100 ml. of toluene are added. 76 gms. (1 mol) of carbon disulfide are added dropwise to the flask. The temperature is maintained within the range of 20 to 30° C. during the addition of the carbon disulfide.

- 5 After the addition, the mixture is refluxed at a temperature of 100  $\pm 10$ ° C. and maintained at this temperature until no further evolution of  $\text{H}_2\text{S}$  is noted. The reaction mixture is cooled to room temperature and the toluene solvent is removed by distillation in vacuo with trace removal of toluene and unreacted amine. The compound



is thereby obtained. One mol of this product is reacted with 0.5 mol (63 gms.) of manganese chloride dissolved in a minimum amount of hot isopropyl alcohol. The mixture is cooled to room temperature and excess alcohol stripped from the reaction product complex. Dichlorobis-N,N'-diphenylthioureamanganese



- 20 is thereby obtained. An analysis of this compound shows 10.5 percent by weight of manganese and 12.2 percent by weight of sulfur.

#### EXAMPLE 16

- 25 To a one liter flask equipped with a stirrer, reflux condenser and dropping funnel, two mols (214 gms.) of benzylamine and 100 ml. of toluene are added. One mol (76 gms.) of carbon disulfide is added dropwise to the flask. During the addition, the temperature is maintained within the range of 20 to 30° C. The mixture is refluxed at 100  $\pm 10$ ° C. until no further evolution of  $\text{H}_2\text{S}$  is noted. The reaction mixture is allowed to cool to room temperature and the toluene solvent removed by distillation in vacuo with trace removal of toluene and unreacted amine. The compound



- 40 is obtained as a reaction product. One mol of this compound is reacted with 0.5 mol (136 gms.) of cadmium bromide dissolved in hot isopropyl alcohol. The mixture is cooled to room temperature and excess alcohol stripped therefrom. Dibromobis-N,N'-dibenzylthioureacadmium ( $\text{Br}_2\text{Cd}[\text{S}=\text{C}(\text{NHCH}_2\text{C}_6\text{H}_5)_2]_2$ ) is obtained as a reaction product.

#### EXAMPLE 17

- 45 Two moles (196 gms.) of cyclohexylamine in toluene are reacted with one mol (76 gms.) of carbon disulfide under reflux conditions. At the cessation of  $\text{H}_2\text{S}$  evolution, the mixture is allowed to cool to room temperature. One mol of the reaction product



- 50 is reacted with 0.5 mols (183 gms.) of cadmium iodide dissolved in a minimum amount of hot isopropyl alcohol. The mixture is cooled to room temperature and excess alcohol stripped from the reaction product complex. Diiodobis-N,N'-dicyclohexylthioureacadmium



65 is obtained as a reaction product.

#### EXAMPLE 18

- 70 To a one liter flask equipped with a stirrer, reflux condenser and dropping funnel, 2 mols (262 gms.) of N'', N'''-dimethyl diethylenetriamine and 100 ml. of toluene are added. One mol (76 gms.) of carbon disulfide is added dropwise at a temperature of 20 to 30° C. The mixture is refluxed until no further  $\text{H}_2\text{S}$  evolution is noted. The reaction mixture is cooled to room tempera-

ture and the toluene subsequently removed. The reaction product obtained has the formula



One mole of this compound is reacted with 0.5 mol (68 gms.) of zinc chloride dissolved in hot isopropyl alcohol. The mixture is cooled to room temperature and excess alcohol stripped therefrom. The complex (dichlorobis - N,N' - di(N'',N'''dimethylidethylene)thioureazinc)  $\text{Cl}_2\text{Zn}[\text{S}=\text{C}(\text{NHC}_2\text{H}_4\text{NHC}_2\text{H}_4\text{N}(\text{CH}_3)_2)_2]_2$  is obtained as a reaction product.

#### EXAMPLE 19

According to the procedures of Example 18, one mol (129 gms.) of N-propylamylamine is reacted with 0.5 mol (38 gms.) of carbon disulfide to produce N,N'-dipropylamylthiourea. 0.5 mol of this product is reacted with 0.25 mol (68 gms.) of cadmium bromide to produce dibromobis-N,N'-dipropylamylthioureacadmium



have been demonstrated to have increased load carrying properties.

Typical examples of these oils including the specific amounts of additive to provide the improved load carrying characteristics will be apparent from the table which follows wherein data is provided on the test results carried out in a standard Shell 4 ball test procedure.

The standard Shell 4 ball test is based on the use of an apparatus that includes 3 rigidly held  $\frac{1}{2}$ " metal balls (type 52-100 steel balls) submerged in the lubricant to be tested in a metal cup. A 4th ball of the same size and material is pressed into contact with the 3 fixed balls by an adjustable loading arm and allowed to rub over a fixed period of time. The contact points on the 3 stationary balls grow to circular scars as wear progresses. The average diameter of these scars in mms after the fixed period of operation at a particular speed and load is taken as a measure of wear. The temperature at which the test is carried out may be varied from room temperature to as high as  $170^\circ\text{C}$ .

Table I.—Extreme pressure properties of lubricating oil compositions determined as seizure and weld in the shell four ball machine (kilograms of load)

| Compound                    | A       |      | B       |      | C       |      | D       |      | E       |      | F       |      |
|-----------------------------|---------|------|---------|------|---------|------|---------|------|---------|------|---------|------|
|                             | Seizure | Weld | Seizure | Weld | Seizure | Weld | Seizure | Weld | Seizure | Weld | Seizure | Weld |
| Plexol 201:                 |         |      |         |      |         |      |         |      |         |      |         |      |
| 0.0.....                    | 55      | 110  | 55      | 110  | 55      | 110  | 55      | 110  | 55      | 110  |         |      |
| 0.3.....                    | (1)     | (1)  | 60      | 140  |         |      |         |      |         |      |         |      |
| 0.5.....                    |         |      | 70      | 145  | 60      | 115  |         |      | 50      | 130  |         |      |
| 1.0.....                    |         |      |         |      | 90      | 170  | 120     | 190  | 110     | 170  |         |      |
| 5.0.....                    |         |      |         |      |         |      | 110     | 225  | 110     | 170  |         |      |
| 10.0.....                   |         |      |         |      |         |      |         |      |         |      |         |      |
| 100 Neutral:                |         |      |         |      |         |      |         |      |         |      |         |      |
| 0.0.....                    | 45      | 110  | 45      | 110  | 45      | 110  | 45      | 110  | 45      | 110  | 45      | 110  |
| 1.0.....                    | (1)     | (1)  | (1)     | (1)  | 100     | 175  | 110     | 150  | 70      | 140  | 70      | 155  |
| 5.0.....                    |         |      |         |      | 100     | 190  | 135     | 205  | 120     | 170  | (1)     | (1)  |
| 10.0.....                   |         |      |         |      | 100     | 220  | 175     | 345  | 110     | 210  |         |      |
| Heavy Intermediate Neutral: |         |      |         |      |         |      |         |      |         |      |         |      |
| 0.0.....                    | 65      | 125  | 65      | 125  | 65      | 125  | 65      | 125  | 65      | 125  | 65      | 125  |
| 1.0.....                    | (1)     | (1)  | (1)     | (1)  | 110     | 160  | 120     | 190  | 80      | 150  | 70      | 140  |
| 5.0.....                    |         |      |         |      | 90      | 165  | 170     | 310  | 110     | 210  | 130     | 190  |
| 10.0.....                   |         |      |         |      | (1)     | (1)  | 100     | 370  | 130     | 230  |         |      |

<sup>1</sup> Additive insoluble in base oil.

#### EXAMPLE 20

Dichlorobis-N,N'-dibutylamylthioureazinc  
( $\text{Cl}_2\text{Zn}[\text{S}=\text{C}(\text{N}(\text{C}_5\text{H}_{11})\text{C}_4\text{H}_9)_2]_2$ )

is prepared by reacting one mol of N-butylamylamine with 0.5 mol of carbon disulfide under reflux conditions in the presence of toluene. The reaction product is then reacted with zinc chloride. The final reaction product is obtained by the procedures described hereinbefore.

#### EXAMPLE 21

Dichlorobis-N,N'-dibutylhexylthioureazinc  
( $\text{Cl}_2\text{Zn}[\text{S}=\text{C}(\text{N}(\text{C}_4\text{H}_9)\text{C}_6\text{H}_{13})_2]_2$ )

is prepared by reacting one mol (157 gms.) of N-butylhexylamine with 0.5 mol (38 gms.) of carbon disulfide under reflux conditions in the presence of toluene. 0.5 mol of the disubstituted thiourea product is then reacted with 0.25 mol of zinc chloride. The final reaction product is obtained by the procedures previously described.

As has been previously indicated the organo-metallic compounds of the present invention unexpectedly provide extreme pressure characteristics for lubricating compositions when added to the same. It has been pointed out that the compounds of the present invention may be added to various mineral and synthetic base stocks in amounts of from .05 to 15 weight percent and preferably from 0.10 to 10.0% by weight. Lubricant compositions prepared with varying amounts of these compounds

In the foregoing table Plexol 201 is the synthetic lubricant (2-Ethylhexyl Sebacate manufactured by Rohm & Haas, Philadelphia, Penn. The 100 Neutral is a base mineral oil having an API gravity of 32 (min.) specific gravity (max.) 0.8654; flash COC °F. (min.) 380; fire COC °F. (min.) 430; viscosity—SUS at  $100^\circ\text{F}$ . 100-110; at  $210^\circ\text{F}$ . 40; VI range (min.) 95 and pour point °F. (max.) 0. The Heavy Intermediate base stock used has the following specification—API gravity 28 (min.), specific gravity (max.) 0.8871; flash COC °F. (min.) 510, fire COC °F. (min.) 570; viscosity—SUS at  $100^\circ\text{F}$ . 632-712; at  $210^\circ\text{F}$ . 70-74; VI range (min.) 95 and pour point °F. (max.) 5.

Referring to Table I, it will be noted that the addition of comparatively small amounts of the new compounds of the present invention substantially improved in every instance the load carrying and extreme pressure characteristics of the lubricating composition to which added. For example, in the composition of 100 Neutral lubricating oil 1% of Compound C increased the seizure load more than 100% and the weld load approximately 50%. In a like manner the addition of Compound D to 100 Neutral oil in the amount of 1% increased the seizure load over 100% and the weld load approximately 35%. When increased to 5% by weight Compound D increased the load carrying property of 100 Neutral from 45 to 135 and the weld load from 110 to 205. In substantially all other cases similar increases are to be noted.

In the examples which follow, representative samples of lubricant compositions prepared with varying base



## 11

wherein X is chlorine, M is zinc, R and R' are hydrogen and R'' and R''' are  $C_2H_4NHC_2H_4N(CH_3)_2$ .

6. A lubricating composition as claimed in claim 1 wherein X is iodine, M is cadmium, R and R' are hydrogen and R'' and R''' are  $C_6H_{11}$ .

7. A mineral oil lubricating composition having extreme pressure properties comprising a major amount of a mineral oil base material and from about 0.5% to about 15.0% by weight of a compound having the formula



wherein M is a metal selected from the group consisting of zinc, cadmium and manganese, R and R' each represents a substituent selected from the group consisting of hydrogen, alkyl having from 3 to 20 carbon atoms, alicyclic having from 6 to 20 carbon atoms, amine-substituted acyclic having from 2 to 11 carbon atoms, aralkyl having from 7 to 20 carbon atoms and aryl and R'' and R''' each represents a substituent selected from the group consisting of alkyl having from 3 to 20 carbon atoms, alicyclic having from 6 to 20 carbon atoms, amine-substituted acyclic having from 2 to 11 carbon atoms, aralkyl having from 7 to 20 carbon atoms and aryl.

8. A mineral oil lubricating composition as claimed in claim 7 wherein M is zinc, R and R' are hydrogen and R'' and R''' are  $C_6H_5$ .

9. A mineral oil lubricating composition as claimed in claim 7 wherein M is zinc, R and R' are hydrogen and R'' and R''' are  $C_4H_9$ .

10. A mineral oil lubricating composition as claimed in claim 7 wherein M is manganese, R and R' are hydrogen and R'' and R''' are  $C_6H_5$ .

11. A mineral oil lubricating composition as claimed in claim 7 wherein M is zinc, R and R' are  $C_4H_9$  and R'' and R''' are  $C_6H_{13}$ .

12. A mineral oil lubricating composition as claimed in claim 7 wherein M is zinc, R and R' are hydrogen and R'' and R''' are  $C_{18}H_{37}$ .

13. A lubricating composition having extreme pressure properties comprising a major amount of synthetic oil base stock and from about 0.05% to about 15.0% by weight of a compound having the formula



wherein M is a metal selected from the group consisting of zinc, cadmium and manganese, R and R' each represents a substituent selected from the group consisting of hydrogen, alkyl having from 3 to 20 carbon atoms, alicyclic having from 6 to 20 carbon atoms, amine-substituted acyclic having from 2 to 11 carbon atoms, aralkyl

having from 7 to 20 carbon atoms and aryl and R'' and R''' each represents a substituent selected from the group consisting of alkyl having from 3 to 20 carbon atoms, alicyclic having from 6 to 20 carbon atoms, amine-substituted acyclic having from 2 to 11 carbon atoms, aralkyl having from 7 to 20 carbon atoms and aryl.

14. A lubricating composition comprising an oil base stock composition as claimed in claim 13 wherein M is zinc, R and R' are hydrogen and R'' and R''' are  $C_4H_9$ .

15. A lubricating composition comprising an oil base stock composition as claimed in claim 14 wherein M is manganese, R and R' are hydrogen and R'' and R''' are  $C_6H_5$ .

16. A lubricating composition comprising an oil base stock composition as claimed in claim 15 wherein M is zinc, R and R' are  $C_4H_9$  and R'' and R''' are  $C_6H_{13}$ .

17. A lubricating composition having extreme pressure properties comprising a major amount of an oil base material and from about 0.05% to about 15.0% by weight of an additive containing mixed alkyl compounds of the formula:



wherein each of R'' and R''' is alkyl having from about 8 to about 18 carbon atoms, R'' and R''' for each alkyl compound differing from that of the other alkyl compounds in said additive.

18. A lubricating composition having extreme pressure properties comprising a major amount of an oil base material and from about 0.05% to about 15.0% by weight of an additive containing mixed alkyl compound of the formula:



wherein each of R'' and R''' is alkyl having from about 9 to about 11 carbon atoms, R'' and R''' for each alkyl compound differing from that of the other alkyl compounds in said additive.

## References Cited by the Examiner

## UNITED STATES PATENTS

|           |       |                |       |          |
|-----------|-------|----------------|-------|----------|
| 1,938,585 | 12/33 | Estabrooke     | ----- | 260—429  |
| 2,704,745 | 3/55  | Kopp et al.    | ----- | 252—47.5 |
| 2,849,420 | 8/58  | Stevens et al. | ----- | 260—429  |

## OTHER REFERENCES

Engle et al.: B35712IVc/23c, June 21, 1956 (German patent application).

60 DANIEL E. WYMAN, Primary Examiner.